

## UNITED STATES PATENT OFFICE

1,972,082

SURFACE HARDENED CAST IRON ARTICLE  
OF MANUFACTURE

Marie Louis André Babinet, Boulogne-sur-Seine, France, assignor, by mesne assignments, to The Nitricastiron Corporation, a corporation of Delaware

No Drawing. Application June 13, 1931,  
Serial No. 544,291

8 Claims. (Cl. 148—31)

My invention relates to the surface hardening of articles made of cast iron alloys, the hardening being effected by the action of nitrogen-containing compounds, for example, ammonia.

5 It is known that certain cast iron alloys may be hardened on their surface portions by subjecting them to a nitriding treatment, i. e. by heating an article made therefrom at a moderate temperature in contact with ammonia or another nitrogen-liberating compound for a considerable period of time. So far as I am aware, all of the cast iron alloys heretofore used for this purpose have contained aluminum as an essential alloying addition. While aluminum is 10 a desirable element from the standpoint of its ability to promote the formation of a hard nitrided surface on castings containing the same, certain problems arise in preparing cast iron alloys containing aluminum and in the production of castings therefrom.

I have found that cast iron alloys containing no aluminum but possessing good nitriding properties may be prepared within the following range of proportions:

|           |             |
|-----------|-------------|
| 25 Carbon | 2.0 to 4%   |
| Manganese | Up to 1%    |
| Silicon   | 1 to 4%     |
| Chromium  | 1.5 to 3.5% |

30 with the balance principally iron. Tungsten may be present in a proportion not exceeding 2%, and as further additions up to 1% each of one or more of the elements titanium, vanadium and molybdenum may be present.

35 While these alloys do not acquire as high a surface hardness by nitriding as do alloys containing aluminum, it is easy to prepare them and to produce castings therefrom. The following are representative examples of alloys coming 40 within the present invention:

|                 | (a)     | (b)     |
|-----------------|---------|---------|
| Carbon (total)  | 3.32%   | 3.39%   |
| Combined carbon | 2.95%   | 1.99%   |
| Silicon         | 1.20%   | 1.84%   |
| Manganese       | .70%    | .71%    |
| Chromium        | 1.75%   | 1.91%   |
| Titanium        | .28%    | 0       |
| Vanadium        | .45%    | 0       |
| Tungsten        | 1.65%   | 0       |
| Molybdenum      | 0       | .25%    |
| Iron            | Balance | Balance |

Alloy (a) showed a hardness before nitriding of 490 Vickers-Brinell and after nitriding a hardness of 710. Alloy (b) showed a hardness before nitriding of 424 Vickers-Brinell and after nitrid-

ing a hardness of 780. The nitriding treatment applied in both cases consisted in heating the casting in the presence of ammonia gas for a period of 50 hours at 500° C.

In cases where it is desired that the castings produced shall be easily machinable either in their natural or "as cast" condition, or after a suitable heat treatment preliminary to the nitriding operation, the silicon content should be raised, so that it will about equal or exceed the percentage of chromium or of chromium and tungsten when the latter is also present.

In nitriding articles made from alloys within the foregoing range of proportions, it is advantageous to subject the article to a preliminary heat treatment to bring the metal into the sorbitic state. This result may be obtained by heating the article to a temperature of around 950° C. and then quenching in a salt bath that has been heated to about 200° C. This treatment may be followed by a re-heating treatment at a lower temperature if desired, although ordinarily the heating necessary to effect the nitriding will bring about such further change in the internal structure of the metal as may be desired.

I claim:

1. An article hardened in its surface portions by nitriding and consisting of an aluminum-free cast iron alloy containing from 2.0 to 4% of carbon, of which a part is present in combined form, from 1.5 to 3.5% of chromium, and from 1 to 4% of silicon with the balance substantially all iron.

2. An article hardened in its surface portions by nitriding and consisting of an aluminum-free cast iron alloy containing from 2.0 to 4% of carbon, of which a part is present in combined form, from 1.5 to 3.5% of chromium, from 1 to 4% of silicon, and an effective and substantial amount but not exceeding about 1% each of the metals titanium, vanadium and molybdenum, with the balance substantially all iron.

3. An article hardened in its surface portions by nitriding and consisting of an aluminum-free cast iron alloy containing from 2.0 to 4% of carbon, of which a part is present in combined form, from 1.5 to 3.5% of chromium, from 1 to 4% of silicon, and an effective and substantial amount but not exceeding about 1% of a metal from the group consisting of titanium, vanadium and molybdenum, with the balance substantially all iron.

4. An article hardened in its surface portions by nitriding and consisting of an aluminum-free cast iron alloy containing from 2.0 to 4% of carbon, of which a part is present in combined

- form, from 1.5 to 3.5% of chromium, from 1 to 4% of silicon, and an effective and substantial amount but not exceeding about 2% of tungsten, with the balance substantially all iron.
- 5 5. An article hardened in its surface portions by nitriding and consisting of an aluminum-free cast iron alloy containing from 2.0 to 4% of carbon, of which a part is present in combined form, from 1.5 to 3.5% of chromium, from 1 to 4% of silicon, an effective and substantial amount but not exceeding about 2% of tungsten, and an effective and substantial amount but not exceeding about 1% of a metal from the group consisting of titanium, vanadium and molybdenum, with the balance substantially all iron.
- 10 6. An article hardened in its surface portions by nitriding and consisting of an aluminum-free cast iron alloy containing from 2.0 to 4% of carbon, of which a part is present in combined

20

form, from 1.5 to 3.5% of chromium, from 1 to 4% of silicon, and an effective and substantial amount but not exceeding about 1% of manganese, with the balance substantially all iron.

7. An article hardened in its surface portions by nitriding and consisting of an aluminum-free cast iron alloy containing about 3.32% carbon, of which a part is present in combined form, about 1.20% silicon, about 0.70% manganese, about 1.75% chromium, about .26% titanium, about .45% vanadium and about 1.65% tungsten.

8. An article hardened in its surface portions by nitriding and consisting of an aluminum-free cast iron alloy containing about 3.39% carbon, of which a part is present in combined form, about 1.54% silicon, about .71% manganese, about 1.91% chromium and about 0.25% molybdenum.

MARIE LOUIS ANDRÉ BBINET.

95

25

100

30

105

35

110

40

115

45

120

50

125

55

130

60

135

65

140

70

145

75

150